

## UNITED STATES PATENT OFFICE

2,338,613

## LUBRICANT

John C. Zimmer, Union, N. J., assignor to Standard Oil Development Company, a corporation of Delaware

No Drawing. Application December 2, 1941,  
Serial No. 421,283

3 Claims. (Cl. 252—35)

This invention relates to lubricants, and more particularly to compounded lubricants comprising mineral oil and lead soap.

There are many lubrication problems, such as the lubrication of high-speed gears, roller bearings, gear trains, etc., for which plain mineral oil does not have a sufficiently strong lubricating film, and for such purposes lead soaps have been incorporated into the mineral oil in order to increase the lubricating film strength thereof. One difficulty with the use of such blends, however, is that under some circumstances, such lubricants have a great tendency to foam, especially in the presence of slight amounts of moisture, as in the lubrication of machinery or other industrial equipment where water occasionally becomes splashed onto the moving metal parts being lubricated.

The primary object of the present invention is to prevent the foaming of such lead-soap compounded lubricants.

It has now been found (and this is the primary feature of the present invention) that the foaming of such lead-soap compounded lubricant can be prevented by incorporating a small amount of an aluminum soap into compounded lubricants containing mineral oil and lead soap.

The lubricating oil base stock to be used may be any mineral oil base stock commonly used for such purposes, and may be derived from various types of crudes, such as paraffinic, naphthenic or mixed base crudes. The viscosity range should preferably be from 50 to about 600 seconds Saybolt Universal at 210° F. It is also generally preferable to use a low cold test oil, i. e., one having a pour point below 10° F.

The lead soaps to be compounded with the mineral oil base stock may be any oil-soluble lead soap having the property of greatly increasing the lubricating film strength. Ordinarily it is preferred to use lead soaps of carboxylic acids, such as higher fatty acids, e. g., oleic acid, stearic acid, etc., or of naphthenic acids, preferably those derived from a gas oil cut of petroleum, although, if desired, corresponding naphthenic acids from a kerosene cut may be used. Preferably the amount of lead soap to be compounded into the mineral oil base stock should be about 5-20%, according to the severity of the conditions under which the lubricant is to be used. In general, such compounded lubricants produce lubricating films 5 to 7 times as strong as that of a plain mineral oil of the same viscosity.

The aluminum soap to be incorporated into the above-described compounded lubricants is preferably aluminum stearate, although, if desired, one may use other aluminum soaps, such as the palmitate, oleate, naphthenate, chelate, capryl or hexyl oxy acetate, phthalate, or the aluminum soap of the fatty acids produced by the oxidation

of paraffin wax, or liquid fractions of substantially saturated petroleum hydrocarbons. Also mixtures of these different types of soaps may be used.

5 The amount of such aluminum soaps required to prevent foaming of the lead-soap compounded lubricant will, of course, vary to some extent according to the viscosity and other characteristics of the base stock as well as upon the amount of lead soap blended therein, and upon the severity of the foam-producing tendencies resulting from the particular operating conditions under which the lubricant will be used, such as the speed of rotation of gears, the relative tendency to whip air into the lubricant and the relative amount of contact with moisture. Generally, however, .05-3% of the aluminum soap should be used, and preferably about 0.5-2%.

20 Although it is believed that the invention applies particularly to aluminum soaps as described above, it is believed that the invention applies more broadly to soaps having a trivalent positive ion, so that specifically, iron soaps such as ferric stearate, ferric naphthenate, etc., could be used instead of aluminum soaps, and in the similarly small amounts specified.

25 The advantages of the invention will be readily observed from a consideration of the following table of foaming test data. In these tests, compounded lubricants were prepared by blending 10% by weight of lead soap into a lubricating oil base stock derived from an asphaltic type crude having light, medium, and heavy viscosities. In each case the compounded lubricant was subjected to the foaming test (a tentative standard A. S. T. M. method for determining foaming tendencies of gear oils) which consisted in beating 500 cc. of the lubricant in a Mix-Master using a 7" diameter and 3 1/4" deep mixing bowl, at 500 R. P. M. for fifteen minutes, and measuring the 30 increase in volume, which is, of course, due to the foaming. Then similar tests were made on the same lubricants to which was added a small amount of aluminum stearate, ranging from 1% 35 in lubricant A to 1.5% in lubricant C.

## Use of aluminum stearate to decrease foaming

| 50 | Lubricant | Aluminum stearate | Vis./210° F. | Gain in volume after beating 15 min. at 500 R. P. M. |     | Decrease in foaming |
|----|-----------|-------------------|--------------|------------------------------------------------------|-----|---------------------|
|    |           |                   |              | Per cent                                             | Cc. |                     |
| 55 | A         | 0                 | 110          | 520                                                  | 520 | 33                  |
|    | A         | 1.0               | 110          | 350                                                  | 350 |                     |
| B  | B         | 0                 | 130          | 675                                                  | 675 | 37                  |
|    | B         | 1.25              | 140          | 425                                                  | 425 |                     |
| C  | C         | 0                 | 230          | 425                                                  | 425 | 74                  |
|    | C         | 1.5               | 193          | 110                                                  | 110 |                     |

60 It is noted in the above table that in all three tests A, B, and C, the use of a small amount of

aluminum stearate (from 1% to 1½%) effected a 33-74% decrease in the amount of foaming.

This result is very important from a practical and commercial point of view and is, indeed, quite surprising because it would normally be expected that the addition of an aluminum soap to a lubricant already containing a lead soap would increase rather than decrease the foaming tendencies. Although the theory of the mechanism of the operation of the present invention is not known with certainty, it is believed that the successful results are possibly due to a lowering of the surface tension effected by the aluminum soap.

Other tests using similarly small amounts of aluminum naphthenate indicate that this material is also very effective as a defoaming agent for lead-soap lubricants.

In addition to the above-described primary ingredients of the composition of this invention, other addition agents which are known to the art may also be incorporated, as for instance, high molecular weight hydrocarbon polymers, e. g., polybutene having a molecular weight above 1,000, especially such polymers having a molecular weight above 30,000, pour depressors, such as those made by Friedel-Crafts condensation of chlorinated paraffin wax with naphthalene, of which the material marketed under the trade-name "Paraflo" is representative, sulfurized fatty oils and other products obtained by sulfurization, sulfur-chloride treatment and halogenation of mineral and fatty oils. Other soaps, such as those of sodium, calcium, etc., may be included to obtain special products, and small amounts of glycerine, alcohols, esters, or amines

may be added as modifying agents for the aluminum soaps.

It is not intended that this invention be limited to the particular materials which have been given merely for purposes of illustration, nor unnecessarily by any theory as to the operation of the invention, but only by the appended claims in which it is intended to claim all novelty inherent in the invention as well as the equivalents coming within the scope and spirit of the invention.

I claim:

1. A lubricant comprising a major proportion of a mineral lubricating oil having a viscosity of about 50-600 seconds Saybolt at 210° F., about 5-20% by weight of an oil-soluble lead soap, and about .05-3% of an oil-soluble aluminum soap.

2. A lubricant comprising a major proportion of a mineral lubricating oil base stock having a viscosity of about 50-600 seconds Saybolt at 210° F. and a pour point below 10° F., about 5-20% by weight of an oil-soluble lead soap of a carboxylic acid selected from the group consisting of higher fatty acids and naphthenic acids, and about .05-3% of an oil-soluble aluminum soap of a carboxylic acid selected from the group consisting of higher fatty acids and naphthenic acids.

3. A lubricant comprising a major proportion of a mineral lubricating oil base stock having a viscosity of about 50-600 seconds Saybolt at 210° F. and a pour point below 10° F., about 5-20% by weight of lead oleate, and about 0.5-2% by weight of aluminum stearate.

JOHN C. ZIMMER.